

1

3,148,061  
PHOTOGRAPHIC DIFFUSION TRANSFER PROCESSES EMPLOYING IMAGE RECEIVING LAYERS CONTAINING POLY-4-VINYLPYRIDINE  
Howard C. Haas, Arlington, Mass., assignor to Polaroid Corporation, Cambridge, Mass., a corporation of Delaware  
No Drawing. Filed Aug. 22, 1960, Ser. No. 50,848  
7 Claims. (Cl. 96—29)

This invention relates to photography and more particularly to novel photographic products and processes.

One object of this invention is to provide novel image-receiving elements for use in color diffusion transfer processes.

Another object of this invention is to provide novel color diffusion transfer processes utilizing said image-receiving elements.

Other objects of the invention will in part be obvious and will in part appear hereinafter.

The invention accordingly comprises the several steps and the relation and order of one or more of such steps with respect to each of the others, and the products possessing the features, properties and the relation of elements which are exemplified in the following detailed disclosure, and the scope of the application of which will be indicated in the claims.

For a fuller understanding of the nature and objects of the invention, reference should be had to the following detailed description.

The present invention is particularly related to color diffusion transfer processes. In such processes a sheet of photosensitive material is exposed to create therein a latent image. The latent image is developed and, concurrent with and under the control of this development, an imagewise distribution of color-providing materials is formed. At least a portion of these color-providing materials is transferred by means of an alkaline aqueous processing liquid to a superposed image-receiving layer to form a colored positive image thereon. As examples of such processes, mention may be made of the processes claimed and disclosed in the copending U.S. application of Howard G. Rogers, Serial No. 748,421, filed July 14, 1958, wherein dye developers (i.e., dyes containing a silver halide developing function and capable of developing exposed silver halide) are the color-providing materials; the processes claimed and disclosed in U.S. Patent No. 2,647,049, issued July 28, 1953, to Edwin H. Land, wherein color developers are employed to develop the latent image and color couplers are the color-providing materials; and the processes disclosed in U.S. Patent No. 2,774,668, issued December 18, 1956, to Howard G. Rogers, wherein complete, preformed dyes which are capable of coupling are used as the color-providing substances.

The image-receiving elements used in such processes generally comprise an opaque or transparent support coated with an image-receiving layer of a dyeable material which is permeable to the alkaline aqueous processing solution. In the past, it has been proposed to use film-forming materials such as polyvinyl alcohol and nylons such as N-methoxymethyl polyhexamethylene adipamide as the dyeable materials.

It has now been discovered that by using an image-receiving layer comprising a polyvinylpyridine polymer and especially a poly-4-vinylpyridine polymer, transfer

2

images having good stability and improved density may be obtained.

The image-receiving elements of this invention are particularly useful in color diffusion transfer processes which employ dye developers. The improvements have been especially marked when azo and anthraquinone dye developers are employed. Dye developers, as noted above, are compounds which contain in the same molecule both the chromophoric system of a dye and also a silver halide developing function. They may be further defined as dyes which are silver halide developers. By "a silver halide developing function" is meant a radical capable of developing an exposed silver halide image. Particularly useful dye developers are those in which the silver halide developing function is provided by the presence of a benzenoid developing radical. A preferred benzenoid developing radical in such compounds is a hydroquinonyl radical. Examples of representative dye developers are given in the previously mentioned U.S. application of Howard G. Rogers, Serial No. 748,421. Additional useful dye developers are described in the following pending U.S. applications:

Application Serial No. 612,045, filed September 25, 1956, in the names of Elkan R. Blout, Milton Green and Howard G. Rogers.

Application Serial No. 612,052, filed September 25, 1956, in the names of Milton Green and Howard G. Rogers.

Application Serial No. 612,053, filed September 25, 1956, in the name of Myron S. Simon.

Application Serial No. 612,054, filed September 25, 1956, in the names of Helen P. Husek and Myron S. Simon.

Application Serial No. 612,055, filed September 25, 1956, in the name of Helen P. Husek.

Application Serial No. 755,804, filed August 18, 1958, in the names of Elkan R. Blout, Saul G. Cohen, Milton Green and Myron S. Simon.

Application Serial No. 824,785, filed July 3, 1959, in the names of Elkan R. Blout, Marilyn R. Cohler, Milton Green, Myron S. Simon and Robert B. Woodward.

Application Serial No. 849,727, filed October 30, 1959, in the names of Elkan R. Blout and Myron S. Simon.

Applications Serial Nos. 1,442 and 1,443, both filed January 11, 1960, in the names of Elkan R. Blout, Saul G. Cohen, Milton Green, Howard G. Rogers, Myron S. Simon and Robert B. Woodward.

In color diffusion transfer processes, employing dye developers, a latent silver halide image in a photosensitive element is developed in the presence of the dye developer and, as a result of this development, the dye developer in the exposed areas is oxidized and substantially immobilized. At least a portion of the immobilization is believed to be at least due, in part, to a change in the solubility characteristics of the dye developer upon oxidation and especially as regards its solubility in alkaline solutions. In unexposed and partially exposed areas of the emulsion, the dye developer is unreacted and diffusible, and thus provides an imagewise distribution of unoxidized dye developer, dissolved in the liquid processing composition, as a function of the point-to-point degree of exposure of the silver halide emulsion. At least part of this imagewise distribution of unoxidized dye developer is transferred, by imbibition, to a superposed image-receiving layer or element, said transfer substantially excluding oxidized dye developer. The image-receiving ele-

ment receives a depthwise diffusion, from the developed emulsion, of unoxidized dye developer without appreciably disturbing the imagewise distribution thereof to provide a reversed or positive color image of the developed image.

The novel image-receiving elements within the scope of this invention may be prepared by coating a sheet of a suitable film support such as cellulose acetate, cellulose acetate-coated baryta paper, etc., which may be suitably subcoated for proper adhesion, with a solution, preferably a 3 to 10% solution, comprising the polyvinylpyridine polymer. Such polymers are generally not soluble in water; however, by using a small amount of acid the image-receiving layers may be cast from aqueous solutions. In a preferred embodiment, volatile acids such, for example, as formic, acetic, etc., are used in applying the coatings. Evaporation of such volatile acids after the image-receiving layer is cast renders said image-receiving layer less water sensitive. The coating and drying operations involved may be carried out by methods commonly employed in the art. The polyvinylpyridine polymer may comprise the sole dyeable film-forming material in the image-receiving layer or it may be added to other image-receiving materials, e.g., gelatin, polyvinyl alcohol, etc. Especially useful results have been obtained when the polyvinylpyridine polymers are used in combination with polyvinyl alcohol. When the polyvinylpyridine polymers of this invention are used in combination with other image-receiving materials the ratio of the polyvinylpyridine polymer to the other image-receiving materials may be varied to suit particular needs. Especially good results have been obtained if the polyvinylpyridine polymers comprise 10 to 100% of the dyeable film-forming materials, with the broadest range being suitable, where polyvinyl alcohol is used.

The term "polyvinylpyridine polymers" as used herein refers to polymers which comprise a major portion of vinylpyridine segments and more preferably to homopolymers of a vinylpyridine. As mentioned above, 4-vinylpyridine polymers have been found particularly useful. Such 4-vinylpyridine polymers provide transfer images which are substantially denser than those produced on poly-2-vinylpyridine image-receiving layers.

The polyvinylpyridine polymers for use in the image-receiving layers of this invention may be prepared by polymerization techniques well known to the art. The following example illustrates the preparation of a polyvinylpyridine polymer for use in the image-receiving layers of this invention.

#### EXAMPLE 1

50 gms. of 4-vinylpyridine, 0.63 gm. of benzoyl peroxide and 0.5 gm. of a 25% aqueous solution comprising 0.912 gm. of hide glue and 0.034 gm. of Nekal BA-75 (trade name of General Dyestuff Corporation, N.Y., for a sodium alkyl naphthalene sulfonate), were placed in 100 cc. of distilled water and polymerized for 2 hours at 50° C. under nitrogen, using a high speed stirrer. The resulting mixture was poured into 3 liters of water and the polymeric precipitate was filtered and washed with an excess of water. The polymer was dried under vacuum at 30° C.

The following non limiting examples illustrate the preparation of image-receiving elements within the scope of this invention.

#### EXAMPLE 2

A sheet of subcoated baryta paper was coated with an aqueous solution containing a small amount of acetic acid and comprising:

|                                                                                                                                          | Percent |
|------------------------------------------------------------------------------------------------------------------------------------------|---------|
| Elvanol 72-60 (trade name of E. I. du Pont de Nemours & Co., Wilmington, Delaware for high viscosity, 100% hydrolyzed polyvinyl alcohol) | 2.4     |
| Poly-4-vinylpyridine                                                                                                                     | 0.08    |
| 1-phenyl-5-mercaptopotetrazole                                                                                                           | 75      |

#### EXAMPLE 3

An image-receiving sheet was prepared as in Example 2 except that the aqueous coating solution comprised acetic acid and:

|                      | Percent |
|----------------------|---------|
| Elvanol 72-60        | 2.16    |
| Poly-4-vinylpyridine | 1.08    |

#### EXAMPLE 4

An image-receiving element was prepared as in Example 2 except that the aqueous coating solution comprised acetic acid and:

|                                | Percent |
|--------------------------------|---------|
| Elvanol 72-60                  | 3.6     |
| Poly-4-vinylpyridine           | 1.2     |
| 1-phenyl-5-mercaptopotetrazole | 0.08    |

#### EXAMPLE 5

A sheet of subcoated baryta paper was coated with an aqueous solution comprising:

|                                | Percent |
|--------------------------------|---------|
| Gelatin                        | 2.25    |
| Poly-4-vinylpyridine           | 2.25    |
| Saponin                        | 0.22    |
| 25 Formaldehyde                | 0.015   |
| 1-phenyl-5-mercaptopotetrazole | 0.098   |

#### EXAMPLE 6

An image-receiving element was made up as in Example 30 2 except that the aqueous coating solution comprised acetic acid and:

|                                | Percent |
|--------------------------------|---------|
| Polyvinyl-4-vinylpyridine      | 2.4     |
| 1-phenyl-5-mercaptopotetrazole | 0.04    |

#### EXAMPLE 7

A control image-receiving sheet was prepared by coating a subcoated baryta paper with an aqueous solution comprising:

|                                | Percent |
|--------------------------------|---------|
| Elvanol 72-60                  | 4.8     |
| Sodium perborate               | 0.01    |
| 1-phenyl-5-mercaptopotetrazole | 0.08    |

and a few drops of a nonionic wetting agent.

The image-receiving elements prepared in the above examples, along with the polyvinyl alcohol control, were tested in diffusion transfer processes by using them in processes employing multilayer photosensitive elements prepared in a manner similar to that disclosed in the above-mentioned copending application Serial No. 748,421. In general, the photosensitive elements comprised a support carrying a red-sensitive silver halide emulsion stratum, a green-sensitive silver halide emulsion stratum and a blue-sensitive silver halide emulsion stratum; said emulsion having disposed in separate alkali-permeable layers behind them, respectively, a cyan dye developer, a magenta dye developer and a yellow dye developer. The particular dye developers employed in the photosensitive elements were (1) 1,4-bis-[ $\alpha$ -methyl- $\beta$ -(2',5'-dihydroxyphenyl)-ethylamino]-5,8-dihydroxyanthraquinone (a cyan dye developer), (2) 2-[p-(2',5'-dihydroxyphenyl)-phenylazo]-4-propoxy-1-naphthol (a magenta dye developer) and (3) 1-phenyl-3-n-hexyl carboxamido-4-[p-(hydroquinonyl-ethyl)-phenylazo]-5-pyrazolone (a yellow dye developer).

In conducting the test, areas of the photosensitive elements were exposed to (1) blue and green light only, (2) red and blue light only, (3) red and green light only, (4) totally exposed and (5) subjected to no exposure. After the transfer process, the integral densities in each of these areas were measured by reflectance using red, green and blue filters.

The results, appearing in tabular form below, indicate the improved density obtained using the image-receiving elements of this invention.

## POLYVINYL ALCOHOL CONTROL OF EXAMPLE 7

| Exposure       | Density    |              |             |
|----------------|------------|--------------|-------------|
|                | Red filter | Green filter | Blue filter |
| Blue and green | 1.17       | 0.46         | 0.31        |
| Red and blue   | 0.12       | 0.79         | 0.50        |
| Red and green  | 0.09       | 0.17         | 0.95        |
| Total exposure | 0.05       | 0.08         | 0.10        |
| No exposure    | 1.22       | 1.24         | 1.65        |

## IMAGE-RECEIVING ELEMENT OF EXAMPLE 2

|                |      |      |      |
|----------------|------|------|------|
| Blue and green | 1.46 | 0.55 | 0.38 |
| Red and blue   | 0.08 | 1.04 | 0.62 |
| Red and green  | 0.03 | 0.21 | 1.54 |
| Total exposure | 0.08 | 0.12 | 0.15 |
| No exposure    | 1.34 | 1.61 | 1.94 |

## IMAGE-RECEIVING ELEMENT OF EXAMPLE 3

|                |      |      |      |
|----------------|------|------|------|
| Blue and green | 1.71 | 0.63 | 0.48 |
| Red and blue   | 0.07 | 0.52 | 0.38 |
| Red and green  | 0.04 | 0.15 | 0.75 |
| Total exposure | 0.08 | 0.10 | 0.13 |
| No exposure    | 1.97 | 1.78 | 1.94 |

## IMAGE-RECEIVING ELEMENT OF EXAMPLE 4

|                |      |      |      |
|----------------|------|------|------|
| Blue and green | 1.57 | 0.69 | 0.46 |
| Red and blue   | 0.09 | 0.98 | 0.62 |
| Red and green  | 0.03 | 0.28 | 1.47 |
| Total exposure | 0.08 | 0.12 | 0.15 |
| No exposure    | 1.45 | 1.68 | 1.99 |

## IMAGE-RECEIVING ELEMENT OF EXAMPLE 5

|                |      |      |      |
|----------------|------|------|------|
| Blue and green | 1.62 | 0.65 | 0.61 |
| Red and blue   | 0.13 | 1.0  | 0.74 |
| Red and green  | 0.07 | 0.30 | 1.57 |
| Total exposure | 0.07 | 0.15 | 0.28 |
| No exposure    | 1.83 | 1.79 | 2.21 |

## IMAGE-RECEIVING ELEMENT OF EXAMPLE 6

|                |      |      |      |
|----------------|------|------|------|
| Blue and green | 0.73 | 0.39 | 0.29 |
| Red and blue   | 0.11 | 0.90 | 0.58 |
| Red and green  | 0.04 | 0.16 | 1.30 |
| Total exposure | 0.07 | 0.09 | 0.12 |
| No exposure    | 0.66 | 1.42 | 2.12 |

When the polyvinylpyridines are used in combination with water-sensitive polymers, such, for example, as polyvinyl alcohol, it is preferable to also employ reagents such as hardeners, cross-linking agents, and other reagents which will reduce the water-sensitivity of the resulting layer.

The transfer images produced on the image-receiving element of this invention, in addition to having improved density, also possess improved brightness and gloss as compared to transfer images produced on polyvinyl alcohol alone.

The image-receiving elements of this invention are especially useful in composite film units intended for use in a Polaroid Land Camera, made by Polaroid Corporation, Cambridge 39, Massachusetts, or a similar camera structure such, for example, as the camera forming the subject matter of U.S. Patent No. 2,435,717, issued to Edwin H. Land on February 10, 1948. In general, such composite film units comprise a photosensitive element, an image-receiving element and a rupturable pod containing an aqueous alkaline processing solution. The elements and pod are so associated with each other that, upon processing, the photosensitive element may be super-

55

60

65

## 6

posed on the image-receiving element and the pod may be ruptured to spread the aqueous alkaline processing solution between the superposed elements. The nature and construction of the pods used in such rolls are well known to the art. See, for example, U.S. Patents Nos. 2,543,181 and 2,634,886, issued to Edwin H. Land.

It is apparent that by selecting a film base from among suitable known opaque and transparent materials, reflection or transparent prints may be obtained.

10 It should be noted that other materials useful in the diffusion transfer processes may be incorporated into the image-receiving layer. As examples of such materials, mention may be made of dye mordants, antifoggants, oxidizing agents, and acids and alkalies for pH adjustments.

15 Since certain changes may be made in the above products and processes without departing from the scope of the invention herein involved, it is intended that all matter contained in the above description shall be interpreted as illustrative and not in a limiting sense.

What is claimed is:

1. In a process of forming a photographic image in color, wherein a latent image contained in an exposed silver halide emulsion is developed in the presence of a dye developer, said dye developer being a compound which is both a dye and a silver halide developer, to provide in said emulsion a predetermined distribution of unoxidized dye developer and wherein at least a portion of said distribution of said unoxidized dye developer is transferred by imbibition from said emulsion to an image-receiving layer in superposed relationship with said emulsion to impart to said image-receiving layer a reversed positive dye image of the developed image, the step of transferring said distribution of unoxidized dye developer to an image-receiving layer comprising poly-4-vinylpyridine.

20 2. A process as defined in claim 1 wherein said image-receiving layer comprises gelatin in addition to said poly-4-vinylpyridine.

25 3. A process as defined in claim 2 wherein the ratio of poly-4-vinylpyridine to gelatin is 1 to 1 on a weight basis.

40 4. A process as defined in claim 1 wherein said image-receiving layer comprises polyvinyl alcohol in addition to said poly-4-vinylpyridine.

45 5. A process as defined in claim 3 wherein the ratio of said poly-4-vinylpyridine to polyvinyl alcohol in said image-receiving layer is about 1 to 2 on a weight basis.

60 6. A process as defined in claim 1 wherein said dye developer is an azo dye developer.

50 7. A process as defined in claim 1 wherein said dye developer is an anthraquinone dye developer.

## References Cited in the file of this patent

## UNITED STATES PATENTS

|           |                |               |
|-----------|----------------|---------------|
| 2,448,542 | McQueen        | Sept. 7, 1948 |
| 2,448,552 | Schulze        | Sept. 7, 1948 |
| 2,548,564 | Sprague et al. | Apr. 10, 1951 |
| 2,548,575 | Weyerts        | Apr. 10, 1951 |
| 2,564,726 | Saner          | Aug. 21, 1951 |
| 2,798,063 | Fowler         | July 2, 1957  |
| 2,830,900 | Land et al.    | Apr. 15, 1958 |
| 2,868,077 | Ryan et al.    | Jan. 13, 1959 |
| 2,983,606 | Rogers         | May 9, 1961   |

## FOREIGN PATENTS

|         |        |              |
|---------|--------|--------------|
| 577,021 | Canada | June 3, 1959 |
|---------|--------|--------------|

UNITED STATES PATENT OFFICE  
CERTIFICATE OF CORRECTION

Patent No. 3,148,061

September 8, 1964

Howard C. Haas

It is hereby certified that error appears in the above numbered patent requiring correction and that the said Letters Patent should read as corrected below.

Column 2, line 20, after "748,421" insert -- (now U.S. Patent No. 2,983,606, issued May 9, 1961) --; line 25, after "Rogers" insert -- (now abandoned and replaced by application Serial No. 144,816, filed October 18, 1961) --; line 28, after "Rogers" insert -- (now abandoned and replaced by application Serial No. 165,940, filed January 12, 1962) --; line 30, after "Simon" insert -- (now abandoned and replaced by application Serial No. 196,523, filed May 21, 1962) --; line 33, after "Simon" insert -- (now abandoned and replaced by applications Serial Nos. 197,259 and 197,283, filed May 24, 1962) --; line 35, after "Husek" insert -- (now abandoned and replaced by applications Serial Nos. 192,354 and 192,355, filed May 4, 1962) --; line 38, after "Simon" insert -- (now abandoned) --; line 41, after "Woodward" insert -- (now abandoned and replaced by application Serial No. 233,461, filed October 26, 1962) --; same column 2, line 43, after "Simon" insert -- (now abandoned) --; column 3, line 54, for "0.912" read -- 0.0913 --; column 4, line 33, for "Polyvinyl-4-vinylpyridine" read -- Poly-4-vinyl-pyridine --; line 51, after "421" insert -- (now U.S. Patent No. 2,983,606, issued May 9, 1961) --; same column 4, line 57, for "magenta" read -- magenta --; column 6, line 45, for the claim reference numeral "3" read -- 4 --; line 67, for "June 3, 1959" read -- June 2, 1959 --.

Signed and sealed this 26th day of October 1965.

(SEAL)

Attest:

ERNEST W. SWIDER  
Attesting Officer

EDWARD J. BRENNER  
Commissioner of Patents